

## UNITED STATES PATENT OFFICE

2,176,426

## LUBRICANT

Gus Kaufman and Samuel R. Philson, Beacon,  
N. Y., assignors to The Texas Company, New  
York, N. Y., a corporation of Delaware

No Drawing. Application July 9, 1937,  
Serial No. 152,757

5 Claims. (Cl. 87—9)

This invention relates to lubricants for use under high pressure conditions, and particularly to an extreme pressure lubricant suitable for use in hypoid gears.

It has been found that a very desirable lubricant having extreme pressure characteristics may be compounded from lubricating oil, sulfur and a lead soap when these ingredients are combined in the correct proportions and under proper conditions. The sulfur is preferably combined with the oil at temperatures which will produce a sulfurized oil in which the sulfur is loosely combined but sufficiently bound to prevent separation of the sulfur on storage. This loosely bound sulfur is essential for the production of our improved lubricant, whereby it is intended that the sulfur will be in such a combined form that it will perform its maximum efficiency under extreme pressure service conditions. The lead soap is preferably lead naphthenate and is preferably combined with the sulfurized oil at temperatures such as to incorporate the lead naphthenate into the oil to produce a homogeneous product but at such a temperature, ordinarily lower than that employed in the sulfurizing treatment, that substantially no lead sulfide is formed and the final product is substantially free from precipitated lead sulfide.

The invention will be further understood from the following illustrative example of the preparation of the improved lubricant.

## Formula

## Per cent

|                                                           |    |
|-----------------------------------------------------------|----|
| Sulfur                                                    | 2  |
| Lead naphthenate (commercial)                             | 5  |
| Lubricating oil—80 Saybolt Universal viscosity at 210° F. | 93 |

The lubricating oil and sulfur were charged with agitation to a grease kettle, heated to about 350° F. and the temperature maintained for approximately 3 hours. The resultant sulfurized oil was then allowed to cool to about 230° F. and the lead naphthenate added with continued agitation. After thorough mixing, the product was allowed to cool and stored. A lubricant so prepared withstood a load of over 6000 pounds according to the method prescribed by the Society of Automotive Engineers.

The manner in which the sulfur is combined with the lubricating oil is important in order to give a product which has the desired extreme pressure characteristics. It has been found that when an oil is drastically sulfurized, for example by heating the oil and sulfur to a high tempera-

ture, with or without pressure, that the sulfur is too tightly bound and the product is unsatisfactory. We prefer to conduct the sulfurizing treatment at a temperature of about 350—375° F. with a heating time of 1—3 hours. Higher temperatures, such as in excess of 400° F., produce too much reaction, forming a product which will not withstand the loads encountered in high pressure use. On the other hand, at lower temperatures stability is sacrificed and the sulfur separates on storage, freezing, or under oxidizing conditions. The reaction temperature is therefore correlated with the time to give a loosely combined sulfurized oil which gives the product extreme pressure properties in addition to the required stability on storage.

It is also important in the manufacture of the product of the present invention to incorporate the lead naphthenate into the product under correct conditions whereby the formation of sludge or precipitation of lead sulfide is avoided. It is desirable to add the lead naphthenate to the sulfurized oil at as high a temperature as possible in order to obtain a homogeneous, stable product but the temperature should not reach that at which a sludge or precipitate is encountered. It is preferable to use temperatures of about 220—250° F. and 230° F. being ordinarily about the maximum temperature which can be used although lower temperatures may be employed as long as the resultant product is homogeneous and of satisfactory stability. The lead naphthenate may be a substantially pure product or a commercial product containing, in addition to the lead naphthenate, various quantities of hydrocarbon oils or other diluents. The product used in the above example was a commercial product obtained from petroleum and containing lead naphthenate equivalent to approximately 2% lead oxide (PbO). It is preferable that sufficient lead naphthenate be used, as a commercial product or otherwise, to produce in the final lubricant a lead naphthenate content of about 1—5%. It is to be understood, of course, that the relative proportions of the sulfur and lubricating oil may be varied but it is preferable to maintain the sulfur content relatively low, for example within the range of about 1—3%.

Obviously many modifications and variations of the invention, as hereinbefore set forth, may be made without departing from the spirit and scope thereof, and therefore only such limitations should be imposed as are indicated in the appended claims.

We claim:

1. A process for the preparation of lubricants for use under high pressure conditions, which comprises forming a sulfurized lubricating oil by heating the oil and sulfur to temperatures of about 350-375° F. for sufficient time to combine the sulfur with the oil in a loosely bound form, and then incorporating lead naphthenate in the sulfurized oil at a temperature of about 220-250° F.
2. A process for the manufacture of extreme pressure lubricants, which comprises incorporating sulfur into a lubricating oil while maintaining a temperature of about 350-375° F. for about 15 1-3 hours, reducing the temperature and commingling lead naphthenate with the resultant product at a temperature of about 230° F.
3. A process for the manufacture of lubricants adapted for use in hypoid gears, which comprises 20 sulfurizing a hydrocarbon lubricating oil at a temperature below 400° F. but sufficiently high that the sulfur is combined with oil in a loosely bound but sufficiently combined form that the final product is stable against sulfur separation 25 on storage, and incorporating lead naphthenate in the resultant product at an elevated temperature below 250° F. such that lead sulfide is not precipitated but sufficiently high to form a stable, homogeneous product.
4. A process for the preparation of lubricants of the extreme pressure type, which comprises

subjecting a mineral lubricating oil and sulfur to temperatures of about 350 to 375° F. thereby forming sulfurized oil containing about 2% sulfur in sufficiently loosely bound form to impart to the oil extreme pressure characteristics and 5 sufficiently tightly bound form to impart to the oil stability against separation of sulfur on storage, and then incorporating about 1 to 5% of lead naphthenate into the sulfurized oil at temperatures of about 220 to 250° F. to form a homogeneous product substantially free from precipitated lead sulfide.

5. A process for the preparation of lubricants of the extreme pressure type, which comprises subjecting a heavy mineral lubricating oil and 15 sulfur to temperatures above about 350° F. but below 400° F. in suitable proportions and for a sufficient length of time to form a sulfurized oil containing about 1-3% of sulfur in sufficiently loosely bound form to impart to the oil high extreme pressure characteristics as measured by the SAE method but sufficiently combined form that the final product is stable against sulfur separation on storage, and then incorporating 1-5% of lead naphthenate in the resultant product 25 at an elevated temperature below 250° F. such that lead sulfide is not precipitated but sufficiently high to form a stable homogeneous final product.

GUS KAUFMAN.

SAMUEL R. PHILSON.

30